

March 14, 1939.

F. H. LE JEUNE

2,150,510

APPARATUS FOR FORMING CASTINGS

Filed Sept. 28, 1936

2 Sheets-Sheet 1



FIG. I.



BY *Whittemore, Hubbard & Belknap*  
ATTORNEYS

March 14, 1939.

F. H. LE JEUNE

2,150,510

APPARATUS FOR FORMING CASTINGS

Filed Sept. 28, 1936

2 Sheets-Sheet 2



FIG. 3.



FIG. 4.

INVENTOR

FRANK H. LE JEUNE

BY

Whittemore, Hubbard & Belknap,  
ATTORNEYS

## UNITED STATES PATENT OFFICE

2,150,510

## APPARATUS FOR FORMING CASTINGS

Frank H. Le Jeune, Detroit, Mich., assignor to  
Kelsey-Hayes Wheel Company, Detroit, Mich.,  
a corporation of Delaware

Application September 28, 1936, Serial No. 103,027

1 Claim. (Cl. 22—209)

The invention relates to the manufacture of castings and refers more particularly to the method of forming castings and the apparatus used.

5 Among the objects of the invention are the provision of an improved method and an improved apparatus for the economical manufacture of uniformly good castings. Another object is to reduce the amount of metal to be melted by eliminating long sprues, gates and feed heads and combining the riser with the sprue, gate and feed head. Further objects are to control the velocity of the molten metal entering the mold cavity; to strain the molten metal before it 10 enters the mold cavity; and the provision of an improved construction for carrying out these functions.

These and other objects of the invention will become apparent from the following description, 20 taken in connection with the accompanying drawings, in which

Figure 1 is a plan view of an apparatus for forming castings, showing an embodiment of my invention;

25 Figure 2 is a cross section on the line 2—2 of Figure 1;

Figure 3 is a view similar to Figure 1, showing another embodiment of my invention;

Figure 4 is a cross section on the line 4—4 of 30 Figure 3.

My invention is particularly applicable to the manufacture of copper silicon castings and, as illustrated, these castings are copper silicon combined hub and brake drum castings for use with 35 wheels of motor vehicles made by a well-known manufacturer.

As illustrated in Figures 1 and 2, 1 is a mold comprising the drag 2 and the cope 3, which together form the mold cavity. This mold cavity has the generally vertically extending annular portion 4, the lateral portion 5 connecting into the generally vertically extending portion and leading toward the axis of the mold cavity, and the central generally vertically extending portion 45 6 connecting into the lateral portion. The peripheral cavity portion 4 is adapted to form the annular brake flange of the brake drum, the lateral cavity portion 5 the web of the brake drum, and the central cavity portion 6 the wheel hub. This latter portion extends both above and below its junction with the lateral portion and radial grooves 7 are preferably formed in the mold cavity extending between the lateral portion and that part of the central portion extending below

its junction with the lateral portion to form radial reinforcing ribs.

8 is a ram-up core formed of core material rammed in place in the drag. This ram-up core forms the mold cavity surface at the junction of the peripheral portion 4 and lateral portion 5 and also the outer lower surface of the lateral portion 5 and the laterally inner surface of the peripheral portion 4. The drag has its remaining portion formed of green sand and includes the portion 9 in which the grooves 7 are formed. In addition, there is the preformed core 10 positioned centrally of the mold cavity and extending upwardly therefrom. The cope is formed of green sand 11, which defines the upper and laterally outer surfaces of the mold cavity. In addition, there is the pouring cup 12 in the nature of a preformed core of core material which extends upwardly above the cope and which engages the upper end of the core 10 to position the same 20 within the mold cavity. The molten metal is adapted to be poured into this cup and to pass therefrom into the upper end of the mold cavity and to then flow throughout the cavity to fill the same. The preformed core 10 and the ram-up core 8 have surfaces in the zones of change of direction of the molten metal so that this molten metal will not destroy the shape of the mold cavity or have imbedded therein, at least to any harmful extent, any of the material forming the surface of the mold cavity.

For the purpose of preventing the entrance of slag into the mold cavity and also for the purpose of controlling the velocity of the molten metal entering the mold cavity and in fact reducing the velocity which it would otherwise have, I have provided the strainer 13 at the lower end of the pouring cup 12. This strainer is integral with and in fact forms the bottom of the pouring cup and it serves to position the upper end of the core 10. The strainer is provided with the annular series of substantially vertically extending openings 14 therethrough which register with the upper end of the central portion 6 of the mold cavity. The construction is such that during the pouring the molten metal within the pouring cup serves as a shrink head to supply molten metal to the casting being formed in the mold cavity upon shrinkage of the metal in this mold cavity. Also with this construction slag and other impurities are prevented from entering the mold cavity and further the velocity of the molten metal entering the mold cavity is controlled and preferably reduced from that it would otherwise have if the strainer were not present.

Furthermore, the size of the strainer openings is such that after the casting has been formed it can be readily separated from its shrink head by breaking the individual gates formed in the openings 14 of the strainer. Furthermore, with this method and apparatus, there is a relatively small amount of metal which can be considered scrap and which must be remelted.

The apparatus as illustrated in Figures 3 and 4, is broadly similar to that illustrated in Figures 1 and 2. In this apparatus the preformed core 15 does not extend upwardly through the mold cavity, the combined hub and brake drum assembly being that for a rear wheel. In this apparatus the pouring cup 16 communicates directly at its lower end with the upper portion of the mold cavity. This pouring cup is considerably higher than the pouring cup 12 and the strainer 17 is located substantially midway between its upper and lower ends to provide a shrink head 18 for compensating for shrinkage in the mold cavity and especially in the central or hub forming portion thereof. The strainer is provided with the series of substantially vertically extending openings 19 therethrough and functions in much the same manner as the strainer 13 to control the velocity of the molten metal entering the cavity and also to prevent slag and other foreign or poor material entering the mold cavity. The

30

total area of the openings is such that sufficient molten metal will pass therethrough to maintain the shrink head. The strainer, instead of being formed integral with the pouring cup, is formed separately therefrom of core material 5 and is adapted to rest upon an annular shoulder 20 formed upon the wall of the pouring cup.

What I claim as my invention is:

In a mold for casting brake drums, the combination of a cope and a drag cooperating to form a mold cavity having a generally axially extending brake flange portion, a generally radially extending web portion connecting into said brake flange portion, a generally axially extending hub portion connecting into said web portion, a preformed core positioned centrally of said hub portion and forming a cavity surface therefor, a ram-up annular core positioned adjacent the radially inner side of said brake flange portion and adjacent the junction of the web portion and the brake flange portion and forming cavity surfaces therefor, a preformed pouring cup in said cope, said cup having a strainer forming the bottom of said cup, said strainer being engageable with the upper end of said first mentioned core to 25 position the latter, and green sand portions in other sections of said cope and drag.

FRANK H. LE JEUNE.

30